

## UNITED STATES PATENT OFFICE

2,218,918

## LUBRICATING OIL

Clarence M. Loane, Whiting, and Bernard H. Shoemaker, Hammond, Ind., assignors to Standard Oil Company, Chicago, Ill., a corporation of Indiana.

No Drawing. Application August 31, 1936,  
Serial No. 98,734

7 Claims. (Cl. 252—47)

This invention relates to improvements in lubricating oils, and particularly, to corrosion inhibited lubricating oils.

In order to obtain increased acceleration and increased speed in present day internal combustion engines it has become necessary to increase both the thermal and mechanical stresses in the engine. In many cases this increase in thermal and mechanical stresses has reached a point where the soft low melting alloys, such as Babbitt metal, are no longer sufficiently durable for bearing duty. It has therefore become necessary to use stronger and more durable bearing materials, and within the last few years "hard metal" bearings, such as copper-lead, cadmium-nickel and cadmium-silver bearings have, to a large extent, replaced Babbitt metal bearings. While mechanically the new type of metal bearings has proven satisfactory, there have been an unusually large number of bearing failures due to corrosion. It has also been noted that the corrosion of "hard metal" alloy bearings has been more marked with "highly" refined lubricating oils.

By "highly" refined lubricating oils we mean oils which have been subjected to such a refining process, for example, solvent extraction, that the paraffinicity of the oil is markedly increased. It has been found that "highly" refined lubricating oils cause corrosion of cadmium-silver alloy bearings to the extent of 5 mgs. per cm.<sup>2</sup> and even greater when bearings are submerged for 25 hours or less in an air agitated oil which has been preoxidized at about 340° F. for 25 to 50 hours.

These "highly" refined lubricating oils have a minimum viscosity range of a S. A. E. 10 oil. Our invention contemplates the use of "highly" refined lubricating oils per se or mixtures of "highly" refined lubricating oils, or mixtures of corrosive oils and non-corrosive oils, such as a corrosive oil and lubricating oil fractions from Winkler Crude or crudes of the Winkler type.

It is, therefore, an object of our invention to provide a highly refined motor oil which will not corrode bearings of the cadmium-silver and copper-lead type.

Another object of our invention is to provide a corrosion inhibitor, which, when added to a highly refined lubricating oil, will prevent the corrosion of "hard metal" bearings such as copper-lead and/or cadmium-silver metal bearings and which will not be detrimental to other desirable properties of the motor oil.

A further object of our invention is to provide

a motor oil containing a very small amount of an organic material which will inhibit the corrosion of bearings in internal combustion engines.

We have found that the foregoing objects may be attained by adding to a "highly" refined motor oil up to 1%, but preferably 0.01% to 0.75% of certain organic materials, particularly long straight chain alkyl thiocyanates and/or long straight chain alkyl isothiocyanates having the general formula RSCN or RNCS where R is an alkyl group. Our invention contemplates the use of alkyl thiocyanates having 8 to 14 carbon atoms and preferably the alkyl thiocyanates having 12 carbon atoms in the alkyl radical, or a mixture of alkyl thiocyanates such as dodecyl, octyl, decyl and tetradecyl thiocyanates, but in which the dodecyl thiocyanate predominates. Our invention also contemplates the use of alkyl isothiocyanates having 8 to 14 carbon atoms in the alkyl radical and preferably the alkyl isothiocyanates having 12 carbon atoms in the alkyl radical, or a mixture of alkyl isothiocyanates such as dodecyl, octyl, decyl and tetradecyl isothiocyanates, but in which the dodecyl isothiocyanate predominates.

We have found that a very effective corrosion inhibitor is obtained when dodecyl thiocyanate or a mixture of alkyl thiocyanates, in which the dodecyl thiocyanate predominates besides small amounts of octyl, decyl, and tetradecyl thiocyanates, is heated in a sealed tube at a temperature of about 350° F. for about three days. The resultant product may be used as such or fractions thereof may be employed. The product may be vacuum distilled under about 1 mm. pressure and the first ninety (90%) percent over used as the corrosion inhibitor or we may extract the product with hot alcohol at about 160-180° F. and the alcohol insoluble portion used, although the alcohol soluble portion may also be used as corrosion inhibitor. Other solvents, particularly very low boiling hydrocarbons such as propane may be used.

We believe that by heating the thiocyanates in the above manner, the same are converted to a substantial degree to the isothiocyanates. However, other products may be formed in the heating process and we therefore do not wish to be limited to any theories as to the compounds formed by heating the thiocyanates.

To determine the effectiveness of the above mentioned compounds as corrosion inhibitors in motor oils we have tested the same in a "highly" refined motor oil under severe engine operating

conditions and in laboratory tests simulating as near as possible extreme engine operating conditions. The following types of tests have been used.

5 **Test 1.**—In this test a "highly" refined oil, to which the corrosion inhibitor is to be added, is preoxidized for either 25 hours or 50 hours by air agitating the same at about 341° F. The corrosion inhibitor and the weighed bearings are placed in the preoxidized oil and the oil air-agitated at about 341° F. The bearings are removed at periodic intervals, washed free of oil and the loss in weight determined.

15 **Test 2.**—In this test the weighed bearings are placed in a "highly" refined oil containing the inhibitor and is air agitated at about 341° F. At periodic intervals the bearings are removed from the oil bath, washed free of oil and the loss in weight determined. Each time before being 20 replaced in the oil bath the bearings are polished bright and reweighed and again tested for predetermined periods. This test differs from test No. 1 in that the test is started with an un-oxidized "highly" refined oil and the test bearings 25 are polished at predetermined intervals.

20 **Test 3.**—In this test the oil containing the corrosion inhibitor is tested in a six cylinder internal combustion engine operating under severe conditions of 2500 R. P. M. at 25 B. H. P. output with 30 a water outlet temperature of about 180° F. and an oil sump temperature of about 320° F. The length of operation before bearing failure is a measure of the effectiveness of the corrosion inhibitor.

35 In each of the above tests the oil used was a motor oil refined to such an extent that a loss in weight of more than 5 mg. per cm.<sup>2</sup> is obtained in 25 hours or less on a cadmium-silver alloy bearing submerged in an air agitated oil at 340° F., which 40 oil has been preoxidized for 25-50 hours at about 340° F.

43 Table I shows the effectiveness of 0.2% of lauryl thiocyanate in a highly refined motor oil as evaluated by Test 1 described above.

Table I

| 50                                  | Hours of test |      |     |    |    |     |
|-------------------------------------|---------------|------|-----|----|----|-----|
|                                     | 3             | 20   | 24  | 48 | 72 | 96  |
| <i>Loss in mgs./cm.<sup>2</sup></i> |               |      |     |    |    |     |
| Control (preoxidized 50 hrs.)       | 6.0           | 41.6 |     |    |    |     |
| Control+0.2% lauryl thiocyanate     | 0.0           | 0.0  | 0.9 |    |    | 5.7 |

55 In Table II are tabulated the results obtained with lauryl thiocyanate and lauryl isothiocyanate as evaluated by Test 1 with a 25 hour preoxidized oil.

Table II

| 60                                  | Hours of test     |     |
|-------------------------------------|-------------------|-----|
|                                     | 6                 | 16  |
| <i>Loss in mgs./cm.<sup>2</sup></i> |                   |     |
| Control (preoxidized 25 hours)      | Corrosion started | 8.1 |
| Control+0.2% lauryl thiocyanate     | do                | 1.1 |
| Control+0.2% lauryl isothiocyanate  | 0.0               | 0.4 |

70 The above results demonstrate the effectiveness of the alkyl thiocyanates and alkyl isothiocyanates of the hereinbefore mentioned type in preventing the corrosion of cadmium-silver 75 bearings.

In Table III we have tabulated results obtained by test method No. 2 described above.

Table III

|                                    | Periods        |               |                |               |
|------------------------------------|----------------|---------------|----------------|---------------|
|                                    | 1st<br>24 hrs. | 2nd<br>6 hrs. | 3rd<br>16 hrs. | 4th<br>6 hrs. |
| Control (fresh oil)                | 2.59           | 5.06          | 20.5           |               |
| Control+0.2% lauryl isothiocyanate | 0.23           | 0.03          | 0.12           | 8.0           |

15 In the engine tests described above as Test No. 3 the effectiveness of the corrosion inhibitors in an oil has been tested in a six cylinder engine operating at 2500 R. P. M. with a 25 B. H. P. output and a water outlet temperature of about 180° F. The oil sump was maintained at a temperature of about 320° F. Using a highly refined S. A. E. 20 oil containing 0.5% of lauryl thiocyanate the bearing failed in 19½ hours. With 0.5% of lauryl isothiocyanate in a sample of the same oil the engine ran for 35 hours without bearing failure. With a sample of the same oil containing no corrosion inhibitor the bearings failed in 12 hours. It should be observed that the above operating conditions are much more severe than those encountered under average actual driving conditions. Under average driving conditions the bearings would last much longer.

20 While we have illustrated our invention in connection with the foregoing examples, we do not wish to limit our invention to the same. These examples are merely illustrative and not a limitation upon the scope of our invention.

25 Where used hereinbefore and in the appended claims, the term lauryl thiocyanate is used to define an alkyl thiocyanate having 8 to 14 carbon atoms in the alkyl chain but predominantly a dodecyl thiocyanate with small amounts of octyl, decyl, and tetra decyl thiocyanate. The term lauryl isothiocyanate as used hereinbefore and in the appended claims is used to define the isothiocyanate of the above compounds.

30 We claim:

1. The method of preventing the corrosion of bearing metal alloys selected from the group consisting of cadmium-silver, cadmium-nickel and copper-lead alloys in the presence of a highly refined lubricating oil normally corrosive to said metal alloys in internal combustion engines which comprises adding to said lubricating oil a substantial amount but not more than 1% of an alkyl thiocyanate having 8 to 14 carbon atoms in the alkyl radical.

35 2. The method of preventing the corrosion of bearing metal alloys having the corrosive susceptibility of alloys of the class consisting of cadmium-silver, cadmium-nickel and copper-lead alloys in the presence of a highly refined lubricating oil normally corrosive to said bearing metal alloys in internal combustion engines which comprises adding to said lubricating oil from about 0.01% to about 1% of an alkyl isothiocyanate having 8 to 14 carbon atoms in the alkyl radical, whereby said highly refined lubricating oil is rendered non-corrosive to said bearing metal alloys.

40 3. The method of preventing the corrosion of bearing metal alloys having the corrosive susceptibility of alloys of the class consisting of cadmium-silver, cadmium-nickel and copper-lead alloys in the presence of a highly refined

lubricating oil in internal combustion engines which comprises adding to said lubricating oil a substantial amount but not more than about 1% of a mixture of alkyl thiocyanates having more than seven carbon atoms in each alkyl radical, said mixture of alkyl thiocyanates comprising predominately dodecyl thiocyanates and small amounts of octyl, decyl, and tetradecyl thiocyanates, whereby said highly refined lubricating oil is rendered non-corrosive to said bearing metal alloys.

4. The method of preventing the corrosion of bearing metal alloys having the corrosive susceptibility of alloys of the class consisting of cadmium-silver, cadmium-nickel and copper-lead alloys in the presence of a highly refined lubricating oil normally corrosive to said bearing metal alloys in internal combustion engines which comprises adding to said lubricating oil from about 0.01% to 1% of a mixture of alkyl isothiocyanates having more than seven carbon atoms in each alkyl radical, said mixture of alkyl isothiocyanates comprising predominantly dodecyl isothiocyanates and small amounts of octyl, decyl, and tetradecyl isothiocyanates, whereby said highly refined lubricating oil is made non-corrosive to said bearing metal alloys.

5. The method of preventing the corrosion of bearing metal alloys having the corrosive susceptibility of alloys of the class consisting of cadmium-silver, cadmium-nickel and copper-lead alloys in the presence of a highly refined lubricating oil normally corrosive to said bearing metal alloys in internal combustion engines which comprises adding to said lubricating oil a substantial amount but not more than about 1% of an organic compound selected from the group consisting of an alkyl thiocyanate having 8 to 14 carbon atoms in the alkyl radical and an alkyl isothiocyanate having 8 to 14 carbon atoms in the alkyl radical whereby corrosion of said bear-

ing metal alloys by said highly refined lubricating oil is inhibited.

6. The method of preventing the corrosion of bearing metal alloys having the corrosive susceptibility of alloys of the class consisting of cadmium-silver, cadmium-nickel and copper-lead alloys in the presence of a highly refined lubricating oil normally corrosive to said bearing metal alloys in internal combustion engines which comprises adding to said lubricating oil from about 0.01% to 1% of an organic compound selected from the group consisting of a mixture of alkyl thiocyanates having more than seven carbon atoms in each alkyl radical, said mixture of alkyl thiocyanates comprising predominately dodecyl thiocyanates and small amounts of octyl, decyl and tetradecyl thiocyanates, and a mixture of alkyl isothiocyanates having more than seven carbon atoms in each alkyl radical, said mixture of alkyl isothiocyanates comprising predominately dodecyl isothiocyanates and small amounts of octyl, decyl and tetradecyl isothiocyanates whereby corrosion to said bearing metal alloys by said highly refined lubricating oil is inhibited.

7. A method of lubricating bearing surfaces which comprises maintaining between metallic bearing surfaces, one of which is an alloy containing a characterizing proportion of a metal selected from cadmium-silver, copper, lead and nickel, a film of lubricating oil normally effective to provide lubrication of the bearing surfaces but which would normally tend to corrode the surface of the aforesaid alloy, said lubricating oil having incorporated therein dodecyl isothiocyanate, in small amount sufficient substantially to retard corrosion of the surfaces of said alloys by said oils.

CLARENCE M. LOANE.  
BERNARD H. SHOEMAKER.